

## UNITED STATES PATENT OFFICE

1,999,134

## HEAT TREATED OILED FILAMENT

Vernon R. Pallas, Cortland, N. Y.

No Drawing. Application November 8, 1932.  
Serial No. 641,739

10 Claims. (Cl. 91—70)

This invention relates to an improved heat treating process for producing a tenacious and relatively pliant filler medium consisting of solidified drying oil or successively applying a series 5 of such coatings to fibriform substances such as threads, strands or braided cords, also textile products of silk, cotton, linen, paper or other materials of this kind likely to suffer serious deterioration when subjected for a prolonged 10 period to temperatures in excess of 200° C., and which process is particularly adapted for the treatment of fish lines and fabrics. The present method is preferably carried out at a controlled elevated temperature in order to speed 15 up production but only for a definitely restricted total period of time which is herein deliberately terminated prior to permitting the tensile strength of the fibriform substance to become inordinately weakened because of such intensified heat application.

My filler medium is purposely kept reasonably free from chemical driers, pigments, gums or other detrimental adulterants likely to produce additional injurious effects upon the solidified 20 drying oil. By virtue of a supplemental seasoning bake, the resulting solidified coating is made to withstand aging without significant hardening or checking, and which step further improves 25 its kink resisting qualities.

The primary object of my invention is to perfect a method of the character indicated capable 30 of rapidly and uniformly processing fibrous substances with one or more successively baked coatings without serious injury to the heat treated 35 fibrous material, also to overcome certain other intrinsic difficulties heretofore encountered in fabricating superior fish lines, textiles or the like oil coated goods on a quick drying productive scale.

The present method is further directed to certain process steps adapted to impart a pliant solidified impregnation or coating to cords, fabrics, or the like, and which steps are performed 40 at a controlled processing temperature ranging between 100° C. and 200° C. Several oil coatings 45 may be superimposed upon an impregnated fibrous substance and each of the respective coatings subjected to a separate baking period sufficient to solidify the drying oil throughout the 50 body thereof. The aim of the present invention lies in utilizing the maximum safe production rate to which such repeated oxidation may be forced and still preserve the tensile strength 55 of the fibrous filament while exposed to intensive heat treatment.

I purposely carry out all of my successive oxidation steps at a comparatively high temperature, having found as the result of extensive research work, that such elevated heat treatment greatly expedites the so-called drying process 5 and makes for a tougher solidified coating that may be properly oxidized throughout the body thereof without resort to chemical drying agents or other accelerators. I have further found that silk and the like line strands were not vitally 10 impaired in tensile strength when subjected to the prescribed temperature range of from 100° C. up to 200° C. for a limited total time period.

From a commercial standpoint, it is advisable to hasten said drying process but if carried on at 15 an excessive rate, this objective may lead to serious deterioration on part of the heat treated strand material. The use of a relatively low processing temperature, i. e., below 100° C., has proven too slow and expensive to satisfy modern 20 productive needs. As deduced from certain laboratory tests conducted upon dry or unimpregnated pure silk fish lines, the strand material thereof when subjected to an oven temperature ranging between 125° C. to 130° C. for an 25 initial period of about sixteen hours, suffered no appreciable drop in tensile strength while being heat treated. Subsequent to such substantially unimpaired dwell period, the loss in material 30 strength gradually dropped in a proportionate relationship with the prolonged time of heat application, showing a deficiency of about 10% in a total time run of 40 hours.

Similar tests made at 150° C. to 155° C. revealed little or no strength impairment during the first 35 hour dwell period but a more pronounced weakening thereafter; the tensile strength originally possessed by the strand material at the beginning of its heat treatment dropped more or less regularly with time and fell to about 35% of such 40 original value in some 40 hours of heat application.

A plot of the test findings pertaining to virgin silk fish line strands, further makes manifest that an oven temperature of from about 140° C. to 45 145° C. still allows a total of six to eight hours in which to successively oxidize and dry applied coatings thereon without inordinate fibre deterioration and a corresponding loss in material strength. On the basis of these same experimental data, the 50 oven temperature may safely be increased in an inversely proportionate relation to the aggregate time of such prolonged heat treatment; where a total of but one or two such coatings are to be applied to a silk strand, my oven temperature 55

may be raised to about 160° C. to 170° C. and still provide for an allowable baking period of about one hour in which to force a correspondingly rapid oxidation of an impregnated strand. When 5 a silk strand is subjected to a processing temperature beyond 200° C., there occurs an immediate and still more decided weakening which provides for substantially no dwell period during which its initial tensile strength is properly up- 10 held.

These comparative test results make apparent that for any given tolerance in strength deterioration, the allowable total time in which to conduct my heat treating process when applied to oil 15 coated filaments, must likewise be shortened in accordance with the particular temperature to which the heat treated strand material is actually subjected. The required successive bakes are preferably so controlled that the aggregate time 20 of heat treatment is appropriately terminated without unduly exceeding the corresponding dwell period to an extent that will allow the tensile strength of the strand material to become seriously impaired.

25 Other materials reach a similar critical reference point upon which to base a suitable raised or lowered baking temperature and a corresponding total baking time. In the case of coating and baking fibrous materials such as cotton, linen, 30 viscose rayon and the like, the prescribed bake period affords ample margin against an inordinate impairment of tensile strength. The maximum allowable baking period is dependent in part upon the characteristic material behavior and the aggregate time to which a given strand may safely 35 be subjected to high drying temperature. All fibrous substances of the kind herein contemplated, undergo a relatively rapid rate of deterioration under prolonged heat treatment when held in excess of 200° C.

40 Referring now to the preferred procedure, an exemplification of my applied process will be directed to the impregnation and heat treating of a fish line or the like product. The usual braided line strand thereof primarily consists of silk material which may initially be kept white or undyed. Such virgin line strand may be impregnated with a filler dope composed in any constituent proportions of suitable raw or treated 45 drying oil such as linseed oil or China wood (tung nut) oil, or the equivalent vegetable or animal drying oils, preferably without the presence of lead, manganese, or the like chemical driers, also reasonably free from pigments or other injurious 50 contaminations likely to weaken the fibrous strand material or injure the quality of its baked coating.

55 After such impregnation, the line strand is transferred to a drying oven containing an oxidizing atmosphere and the strand material is preferably held at a relatively elevated temperature of around 140° C. to 145° C. Under this degree of heat one and one-half hours usually suffice to harden and substantially dry out a fully impregnated fish line strand when using a mixture of equal parts by volume of raw China wood oil and refined linseed oil that is kept free from chemical driers.

60 Thereupon, the line may be repeatedly re- 70 turned to said bath for a like treatment but being more adequately surfaced, each subsequent oil coating normally requires only  $\frac{1}{3}$  to  $\frac{1}{2}$  of the above stipulated drying time, the processing of the respective additional coatings being otherwise 75 identical in method to that given to the initial

strand impregnation. Any number of such coatings or layer courses may be successively applied within the stipulated total baking time until a homogeneous body of solidified drying oil has been built up around the heat treated line strand, 5 which in the case of fine trout fishing lines, may require 8 to 12 consecutive coatings and a corresponding number of bakes. As will be understood, such alternate dipping and drying steps may be facilitated by the use of conventional oven 10 conveyor appliances, and also that surface finishing machinery is commonly used to individually hone up the respective line coatings after being dried.

15 The specified drying temperature range of 100° C. to 200° C. is herein relied upon to accelerate the oxidizing process without requiring chemical driers or the like accelerator agencies. Such adulterants have been found to produce stiffening and other injurious effects upon the finished 20 product. When used in excess, driers of this kind are generally sluggish in wholly completing the oxidation process and their lingering chemical action apparently persists for a long period after the coatings have been baked, thereby causing 25 the aged coating to become brittle with time. For a similar reason, it is preferred not to introduce rosin, gum or pigment into my dope bath prior to subjecting the coatings to high oven 30 temperature. It is further preferred to introduce any needed line coloring matter into the solidified oil coating as an ultimate step, that is to say, after all coating operations thereon have been completed.

35 A further goal is to provide for a durable but pliant solidified coating that shall be suitable as applied to fish line or fabric goods that are expected to be sharply flexed in normal use. A difficulty heretofore met with in successfully providing for such purposes, lies in obliterating the 40 dominating yellow color common to most drying oils without mixing a pigment in the filler dope bath. Unless fortified by the hereinafter prescribed seasoning step, the translucent oil coating is likely to develop a conspicuous localized 45 opaqueness or pronounced change in refractive index when subjected to a sharp kinking test. My process is intended to mitigate or substantially overcome such spotty surface defect by maintaining a more nearly uniform translucency 50 throughout the line length. The cited imperfection is a matter of particular importance as regards the appearance of fine trout fishing lines, since they are normally subjected to hard usage while being cast and likely to become inadvertent- 55 ly kinked.

To this end, I preferably start out with a braided silk strand, and apply thereto successive coatings that are baked in the manner previously specified. As a supplementary step, my oil coated 60 line or fabric may be subjected to a prolonged final bake of from one to three hours at comparatively high temperature preferably ranging between 140° C. to 150° C., which seasoning period serves to more thoroughly complete oxidation 65 without inordinately weakening the fibrous strand, hence additionally toughens and otherwise improves my pliant strand coatings in with- standing a kinking strain.

70 The foregoing is descriptive of a method that has been found wholly satisfactory in practice as applied to the commercial manufacture of fishing line and analogous fibrous products. A fish line made in accordance with my process not only handles well and remains soft and pliable, 75

but to a marked degree solves the cited kinking problem. This objective is preferably secured by working with a strand filler medium kept substantially pure throughout the processing steps and allowing no impurities to be introduced which under intensive heat treatment, may tend to set up secondary or other detrimental chemical reactions. Said process is also admirably suited for the treatment of cloth or other woven goods of suitable texture which may similarly be impregnated and baked to make up table covers, window shades, raincoats, umbrella covers and the like moderately waterproofed sheet materials.

I claim as my invention:

15. 1. The process of treating a fish line and which process comprises coating the one strand with a drying oil substantially free from a chemical drier and baking at a controlled temperature ranging between one hundred degrees centigrade and two hundred degrees centigrade for a limited length of time to solidify the drying oil without substantially impairing the tensile strength originally possessed by the line strand prior to such limited baking period.
25. 2. The process for fabricating a fish line and which process consists in providing for a line strand of material whose tensile strength deteriorates when said strand is subjected to prolonged baking; impregnating said strand with drying oil substantially free from a chemical drier; then baking the impregnated strand in an oxidizing atmosphere; thereupon, applying a coating of drying oil thereon and further baking to solidify the strand coating at a controlled temperature not less than one hundred degrees centigrade and not higher than two hundred degrees centigrade, the aggregate baking time being terminated in accordance with the baking temperature to which the strand is actually subjected, whereby to preserve the tensile strength of the strand material against inordinate deterioration during such successive baking periods.
35. 3. The process for intensively heat treating a fish line and which process consists in providing for a line strand of material whose tensile strength deteriorates when subjected to prolonged baking; impregnating said strand with drying oil; introducing the impregnated strand for a certain period of time into an oxidizing atmosphere to solidify the drying oil at a controlled baking temperature in excess of one hundred degrees centigrade but not higher than two hundred degrees centigrade; and thereupon coating the aforesaid strand with drying oil and further baking the strand material to solidify said coating, the total time of all such baking of the strand material inclusive of said certain period being restricted in accordance with the baking temperature actually employed, and which total time is terminated prior to allowing the tensile strength of the strand material to become substantially impaired while being subjected to such successive heat treatment.
45. 4. The heat treating process which consists in providing for a strand primarily comprised of silk material that is impregnated with drying oil; introducing the impregnated strand for a certain period of time into an oxidizing atmosphere to initially solidify the drying oil at a controlled baking temperature in excess of one hundred and twenty degrees centigrade but not in excess of one hundred and eighty degrees centigrade; and thereupon coating said strand with drying oil and further baking the strand material to solidify said coating, the total time
- allowed for all such baking of the strand material inclusive of said certain period, being terminated in accordance with the baking temperature actually employed and the tensile strength of the strand material being thereby preserved against inordinate deterioration while being subjected to the aforesaid baking temperature.
5. The heat treating process which consists in providing for a strand primarily comprised of silk material that is impregnated with drying oil; baking the impregnated strand in an oxidizing atmosphere; then applying a coating of drying oil thereon and further baking to solidify the strand coating at a controlled temperature held at more than one hundred and twenty degrees centigrade but not in excess of one hundred and eighty degrees centigrade, the aggregate time of all such baking of the strand material being terminated in accordance with the baking temperature actually employed, whereby to preserve the tensile strength of the strand material against inordinate deterioration while being subjected to such successive bakes.
10. 6. The process for improving the kinkproof quality of a fish line and which process consists in providing for a line strand of material whose tensile strength deteriorates when subjected to prolonged baking; coating the strand with semitransparent drying oil and baking said coated strand in an oxidizing atmosphere for a length of time sufficient to solidify the drying oil; and whereupon the solidified coating is kinkproofed by a seasoning step comprising an additional baking at a temperature held to not less than one hundred degrees centigrade nor in excess of two hundred degrees centigrade to render said line capable of withstanding localized kinking strain and of maintaining substantial uniform transparency when subjected to such strain, the aggregate baking time being controlled and terminated in accordance with the baking temperature to which said strand is actually exposed, whereby to complete all of such baking time without inordinate deterioration in tensile strength while the material is being subjected to such successive bakes.
15. 7. A fish line comprising a strand of fibrous material coated with a semitransparent drying oil and which coating has by heat treatment, been converted into a solidified pliant body characterized by its ability to maintain substantial uniform transparency when the coated strand is subjected to a localized kinking strain, said heat treating including a seasoning step baking the solidified drying oil at a temperature ranging between one hundred degrees centigrade and one hundred and eighty degrees centigrade without substantially impairing the tensile strength of the strand material.
20. 8. The process of heat treating a fish line and which process comprises coating the line strand with a drying oil and baking at a controlled temperature ranging between one hundred degrees centigrade and two hundred degrees centigrade for a limited period of time that is terminated in accordance with the baking temperature to which the strand is actually subjected, the tensile strength of the strand material being thereby preserved against inordinate deterioration while exposed to the aforesaid baking temperature.
25. 9. The kinkproofing process which comprises coating a strand of fibrous material with translucent drying oil; then baking said coated strand

- in an oxidizing atmosphere and which baking includes a seasoning period held at a temperature ranging between one hundred degrees centigrade and two hundred degrees centigrade with-  
5 out allowing the tensile strength of the strand material to become unduly impaired during such seasoning period, said seasoning serving to convert the drying oil into a pliant body that maintains substantial uniform translucency when  
10 subjected to a localized kinking strain.
10. The process for heat treating a fish line strand or the like fibriform substance, and which process consists in providing for a strand of material whose tensile strength deteriorates when subjected to prolonged baking; applying a series of drying oil coatings upon said strand and baking the respective strand coatings in an oxidizing atmosphere at a controlled processing temperature not less than one hundred degrees centigrade and not higher than two hundred degrees centigrade, the aggregate baking time being terminated in accordance with the actual processing temperature employed and thereby preserve the tensile strength of the strand ma-  
10 terial against undue deterioration while exposed to such processing temperature during the afore-  
said aggregate time period.

VERNON R. PALLAS.

CERTIFICATE OF CORRECTION.

Patent No. 1,999,134.

April 23, 1935.

VERNON R. PALLAS.

It is hereby certified that error appears in the printed specification of the above numbered patent requiring correction as follows: Page 2, second column, line 7, for "required" read require; page 3, first column, line 16, claim 1, for "one" read line; and that the said Letters Patent should be read with these corrections therein that the same may conform to the record of the case in the Patent Office.

Signed and sealed this 18th day of June, A. D. 1935.

Leslie Frazer

(Seal)

Acting Commissioner of Patents.

## DISCLAIMER

1,999,134.—*Vernon R. Pallas*, Cortland, N. Y. HEAT TREATED OILED FILAMENT.  
Patent dated April 23, 1935. Disclaimer filed January 29, 1940, by the  
patentee.

Hereby enters this disclaimer as follows:

(a) To those parts of the specification in the following words: "also textile products" (p. 1, col. 1, lines 6-7); "paper" (p. 1, col. 1, line 7); "and fabrics" (p. 1, col. 1, line 12); "textiles" (p. 1, col. 1, line 37); "fabrics," (p. 1, col. 1, lines 42-43); "or fabric goods" (p. 2, col. 2, line 37); "or fabric" (p. 2, col. 2, line 61); "Said process is also admirably suited for the treatment of cloth or other woven goods of suitable texture which may similarly be impregnated and baked to make up table covers, window shades, raincoats, umbrella covers and the like moderately waterproofed sheet materials." (p. 3, col. 1, lines 8-13.)

(b) To that part of the specification in the following words: "one or" (p. 1, col. 2, line 54).

(c) To claims 1 and 8;

(d) To all processes described in claims 2, 3, 4, and 5 and each of them except processes in which the impregnated, baked and coated line is subjected to the said further baking for a period of at least one hour.

(e) To all processes described in claim 10 except processes in which the last of the said series of drying oil coatings applied to the line is subjected to baking as described for a period of at least one hour.

[*Official Gazette February 27, 1940.*]

## DISCLAIMER

1,999,134.—*Vernon R. Pallas*, Cortland, N. Y. **HEAT TREATED OILED FILAMENT.**  
Patent dated April 23, 1935. Disclaimer filed October 6, 1942, by the  
patentee.

Hereby enters this disclaimer to claims 2, 3, 4, 5, and 10.  
[Official Gazette November 10, 1942.]